

July 16, 1935.

M. G. JEWETT ET AL

2,008,452

HEAT TREATED CAST IRON AND PROCESS OF PRODUCING THE SAME

Filed Sept. 23, 1931

*Fig. 1.*



MAGNIFIED 1000 DIAMETERS

*Fig. 2.*



MAGNIFIED 1000 DIAMETERS

*Fig. 3.*



MAGNIFIED 1000 DIAMETERS

*Fig. 4.*



MAGNIFIED 1000 DIAMETERS

INVENTORS:  
Maurice G. Jewett and  
Samuel C. Harris,  
BY Barker & Collins  
ATTORNEYS.

## UNITED STATES PATENT OFFICE

2,008,452

HEAT TREATED CAST IRON AND PROCESS  
OF PRODUCING THE SAME

Maurice G. Jewett and Samuel C. Harris,  
Milwaukee, Wis., assignors to Chain Belt  
Company, Milwaukee, Wis., a corporation of  
Wisconsin

Application September 23, 1931, Serial No. 564,634

22 Claims. (Cl. 148—21.7)

This invention relates to processes of treating malleable iron, for the purpose of improving its physical properties, and also imparting thereto the property of being hardened to increase its strength, yield point, and resistance to wear; and is a continuation in part of our application, filed September 17, 1930, Serial Number 482,589.

An object of the invention is to modify the character of the iron-carbon grain composition by appropriate heat treatment, in order to develop a grain having a homogeneous spheroidized cementite pearlitic structure.

A further object of the invention is to develop a surface on malleable cast iron to impart thereto a very high resistance to wear and thereby increase its durability in use, while developing the homogeneous spheroidized cementite grain structure.

Other objects of the invention will be apparent to those skilled in the art.

It is well-known to metallurgists, that while the commercial malleable cast iron obtainable in the open market is considerably more ductile than unmalleabilized cast iron, at the same time it is weak and relatively soft, and lacks desired durability in use. Likewise, although less susceptible to fracture from shocks or loads than ordinary cast iron, it still leaves something to be desired in this respect; the present invention accordingly aims to provide a process of heat treating ordinary malleable cast iron to increase its durability, strength, and utility in the arts.

Accordingly, the invention consists in the novel steps and combinations constituting the process as described herein and particularly pointed out in the appended claims.

In the accompanying drawing, the photomicrographs are all made at the same magnification, 1000 diameters.

Fig. 1 is a copy of a photomicrograph of a polished and etched surface of ordinary malleable cast iron;

Fig. 2 is a copy of a photomicrograph of a polished and etched surface of malleable cast iron after having been subjected to a heat treatment of about 1600° F. for one hour, and immediately drastically cooled, showing a martensitic grain structure;

Fig. 3 is a copy of a photomicrograph of a polished and etched surface of malleable cast iron after having been heat treated to about 1600° F. for one hour, immediately drastically cooled, and again heat treated or tempered at 1325° F. for one hour, and immediately drastically cooled, and

showing a homogeneous spheroidized cementite grain structure; and

Fig. 4 is a copy of a photomicrograph of a polished and etched surface of a commercial type of malleable cast iron after having been heat treated to about 1475° F., then quenched, then reheated to from 900° F. to 1200° F., and again quenched; the illustration exhibits a pearlitic-sorbitic grain structure.

In Fig. 1, which illustrates the physical structure of regular commercial malleable cast iron as produced at the present time, the pure ferrite crystals 1 are illustrated as having thin boundary lines, 2, and also illustrates inclusions, or "islands" of graphitic carbon 3. Upon heating such cast iron to well above its critical or carbon combining point, for example, from about 1475° F. to about 1600° F. or higher, which may be in the presence of a carburizing agent to increase the carbon content of the outside surface 10 of the iron which has been previously decarburized, for a sufficient length of time, about one hour or longer depending upon the mass of the iron, to allow the ferrite grain to absorb or combine with variable quantities of carbon from the 15 associated graphite and form an iron carbide, for example, from about one-tenth percent to about one percent of carbon, and then immediately drastically quenching, by immersion in oil or water to a point below about 900° F., or very materially below its carbon combining temperature, 20 the ferrite grains will combine with carbon and will have been converted into a martensitic structure as shown at 4 in Fig. 2, and the product will be very wear-resisting. The length of 25 time the metal is held at a temperature above the critical point will determine the percentage of graphitic carbon combined with the ferrite, and the characteristics of this martensitic structure will be controlled by the percentage of carbon absorbed by the ferrite crystals. Disregarding the inclusions, or "islands" of graphite 3, the 30 cast iron thus treated will have a structure corresponding to that of a carbon steel of like percentage of carbon absorption, and in heat treatment will respond to the same general rules that govern the tempering of steel of like carbon content.

Upon reheating the cast iron having the structure illustrated in Fig. 2, to a temperature from about 1300° F. to about 1325° F., or slightly higher, for about one hour, (which is just below the critical point range, about 1350° F. to about 1450° F.) and then immediately drastically quenching in oil to about 900° F. or lower, the 50 55

iron will possess the greatest ductility with the maximum increased strength, and will have its grain composition converted into a homogeneous spheroidized cementite pearlitic structure as illustrated at 5, in Fig. 3, but not into the sorbitic structure illustrated in Fig. 4; and disregarding the graphite inclusions, the structure illustrated in Fig. 3 resembles the analogous pearlitic-spheroidal-cementite structure that is exhibited by steel of like carbon content produced in the regular commercial way.

A known grade of iron, produced by heating malleable cast iron to about 1475° F. for a sufficient time, and then quenching in oil, water, or other medium, and then reheating to from 900° F. to about 1200° F. produces a product having a grain structure as illustrated in Fig. 4, in which the martensitic structure has been converted into a pearlitic-sorbitic structure shown at 6. The iron produced by the treatment in accordance with the present invention, by a first heating to about 1600° F., then immediately drastically cooling, and then a second heating to 1325° F. and immediately drastically cooling, does not produce a grain having a sorbitic structure, but on the contrary produces a grain having a homogeneous spheroidized cementite pearlitic structure illustrated at 5 in Fig. 3, as above noted which has about twenty percent greater strength than the pearlitic-sorbitic structure, with a corresponding increase in yield point, and a combined carbon content from about 0.50 percent to about 0.85 percent, a Brinell hardness from about 145 to about 217, a tensile strength of from about 75,000 pounds to 90,000 pounds per square inch, and an elongation of from about five percent to about 13 percent, and the most desirable machining qualities.

Upon heating specimens of malleable cast iron to different temperatures above its critical or carbon combining point, and then drastically quenching in oil to considerably below its critical point, and then reheating to about 1325° F. and again drastically quenching in oil and cooling to normal temperatures, the specimens possessed the following characteristics—

1

Heat to 1475° F., and drastically quench in oil;  
Reheat to 1325° F., and drastically quench in oil;  
Combined carbon .48%  
Brinell 143  
Tensile strength 75,650 pounds per sq. in.  
Elongation 13%

2

Heat to 1525° F., and drastically quench in oil;  
Reheat to 1325° F., and drastically quench in oil;  
Combined carbon .54%  
Brinell 149  
Tensile strength 84,200 pounds per sq. in.  
Elongation 9%

3

Heat to 1600° F., and drastically quench in oil;  
Reheat to 1325° F., and drastically quench in oil;  
Combined carbon .82%  
Brinell 217  
Tensile strength 90,000 pounds per sq. in.  
Elongation 5%

The treatment of malleable cast iron by the processes of the present invention produces a

product having the characteristics indicated in the examples, given above, having a combined carbon content of from 0.50% to 0.85%, and a Brinell hardness of 145 and upwards with excellent machining qualities, and with an ultimate strength and yield point of from about 75,000 pounds to about 87,000 pounds, and upwards, per square inch.

Malleable iron, as the term is used in this specification and claims, refers to any cast iron which has the property of malleability; one example thereof being where such property, as an end result, has been developed through heat treatment of a metal such as the so-called white iron, which in most cases has no appreciable malleability prior to such heat treatment. However, as in ordinary commercial usage, such cast irons are to be clearly distinguished from steel, which is also an iron product possessing malleability. The present claims are not intended to extend to this latter class of iron products, but only to cast irons as that term is ordinarily understood in the art.

While for purposes of the present disclosure whereby others may be enabled to practice the invention, one particular example has been described, it will be obvious that those skilled in the art to which it appertains may vary the details thereof without departing from the gist of the invention, which is the production of a heat treated cast iron having a homogeneous spheroidized cementite matrix structure, with the major portion of the carbon being in the graphitic form; and therefore it is not wished to be limited to the above disclosure except as may be required by the appended claims.

We claim:—

1. The method of developing in malleable cast iron, a grain having a homogeneous spheroidized cementite pearlitic structure, substantially free from sorbitic structure, which comprises subjecting malleabilized cast iron to a temperature from about 1475° F. to about 1600° F. for a time sufficient to combine with associated carbon, then drastically cooling to form a martensitic structure, then reheating to about 1325° F. for a time sufficient to convert said martensitic structure into a homogeneous spheroidized cementite pearlitic structure substantially free from sorbitic structure, and again drastically cooling.

2. The method of developing in malleable cast iron, a grain having a homogeneous spheroidized cementite pearlitic structure, substantially free from sorbitic structure, which comprises subjecting malleabilized cast iron to a temperature from about 1475° F. to about 1600° F. for not less than one hour, then drastically cooling to form a martensitic structure, then reheating to about 1325° F. for not less than one hour to convert said martensitic structure into a homogeneous spheroidized cementite pearlitic structure substantially free from sorbitic structure, and again drastically cooling.

3. The method of developing in malleable cast iron, a grain having a homogeneous spheroidized cementite pearlitic structure, substantially free from sorbitic structure, and developing in the treated iron a strength of 87,000 pounds and upwards per square inch, which comprises subjecting malleabilized cast iron to a temperature of about 1600° F. for a time sufficient to combine with associated carbon, then drastically cooling to form a martensitic structure, then reheating to about 1325° F. for a time sufficient to convert said martensitic structure into a homogeneous spheroidized cementite pearlitic structure substantially

free from sorbitic structure, and again drastically cooling.

4. The method of developing in malleable cast iron, a grain having a homogeneous spheroidized cementite pearlitic structure, and developing in the treated iron a strength of 87,000 pounds and upwards per square inch, which comprises subjecting malleabilized cast iron to a temperature of about 1600° F. for not less than one hour, then 5 drastically cooling to form a martensitic structure, then reheating to about 1325° F. for not less than one hour to convert said martensitic structure into a homogeneous spheroidized cementite pearlitic structure, and again drastically cooling.

15 5. The method of developing in malleable cast iron, a grain having a homogeneous spheroidized cementite pearlitic structure, and having a combined carbon content of from about 0.50 percent to about 0.85 percent, which comprises subjecting malleabilized cast iron to a temperature of about 1600° F. for a time sufficient to combine with associated carbon, then drastically cooling to form a martensitic structure, then reheating to from 1300° F. to about 1325° F. for a time sufficient 20 to convert said martensitic structure into a homogeneous spheroidized cementite pearlitic structure, and again drastically cooling.

6. The method of developing in malleable cast iron, a grain having a homogeneous spheroidized cementite pearlitic structure, substantially free from sorbitic structure, and having a combined carbon content of from about 0.50 percent to about 0.85 percent, which comprises subjecting malleabilized cast iron to a temperature of about 35 1600° F. for not less than one hour, then drastically cooling to form a martensitic structure, then reheating to about 1325° F. for not less than one hour to convert said martensitic structure into a homogeneous spheroidized cementite pearlitic structure substantially free from sorbitic structure, and again drastically cooling.

7. The method of developing in malleable cast iron, a grain having a homogeneous spheroidized cementite pearlitic structure, substantially free from sorbitic structure, and having a combined carbon content of from about 0.50 percent to about 0.85 percent and upwards, which comprises subjecting malleabilized cast iron to a temperature of about 1600° F. in a carburizing 50 environment for a time sufficient to combine with associated carbon, then drastically cooling to form a martensitic structure, then reheating to about 1325° F. for a time sufficient to convert said martensitic structure into a homogeneous spheroidized cementite pearlitic structure substantially free from sorbitic structure, and again drastically cooling.

8. The method of developing in malleable cast iron, a grain having a homogeneous spheroidized cementite pearlitic structure, substantially free from sorbitic structure, and having a combined carbon content of from about 0.50 percent to about 0.85 percent, which comprises subjecting malleabilized cast iron to a temperature of about 65 1600° F., in a carburizing environment, for not less than one hour, then drastically cooling to form a martensitic structure, then reheating to about 1325° F. for not less than one hour to convert said martensitic structure into a homogeneous spheroidized cementite pearlitic structure substantially free from sorbitic structure, and again drastically cooling.

9. The method of developing in malleable cast iron, a grain having a homogeneous spheroidized cementite pearlitic structure, substantially free

from sorbitic structure, and developing in the treated iron a strength of 87,000 pounds and upwards per square inch, and a Brinell hardness of 200 and upwards, which comprises subjecting malleabilized cast iron to a temperature of about 1600° F. for a time sufficient to combine with associated carbon, then drastically cooling to form a martensitic structure, then reheating to about 1325° F. for a time sufficient to convert said martensitic structure into a homogeneous 10 spheroidized cementite pearlitic structure substantially free from sorbitic structure, and again drastically cooling.

10. The method of developing in malleable cast iron, a grain having a homogeneous spheroidized cementite pearlitic structure, substantially free from sorbitic structure, and developing in the treated iron a strength of 87,000 pounds and upwards per square inch, and Brinell hardness of 200 and upwards, which comprises subjecting 15 malleabilized cast iron to a temperature of about 1600° F. for not less than one hour, then drastically cooling to form a martensitic structure, then reheating to about 1325° F. for not less than one hour to convert said martensitic structure into 20 a homogeneous spheroidized cementite pearlitic structure substantially free from sorbitic structure, and again drastically cooling.

11. The method of developing in malleable cast iron, a grain having a homogeneous spheroidized cementite pearlitic structure, substantially free from sorbitic structure, and having a combined carbon content of from about 0.75 percent to about 0.85 percent, a strength of about 87,000 pounds and upwards per square inch and a 30 Brinell hardness of about 200 and upwards, which comprises subjecting malleabilized cast iron to a temperature of about 1600° F. for a time sufficient to combine with associated carbon, then drastically cooling to form a martensitic structure, then reheating to about 1325° F. for a time sufficient to convert said martensitic structure into a homogeneous spheroidized cementite pearlitic structure 35 substantially free from sorbitic structure, and again drastically cooling.

12. The method of developing in malleable cast iron, a grain having a homogeneous spheroidized cementite pearlitic structure, and having a combined carbon content of from about 0.65 percent to about 0.85 percent, a strength of about 87,000 pounds and upwards per square inch and a Brinell hardness of about 200 and upwards, which comprises subjecting malleabilized cast iron to a temperature of about 1600° F. for not less than 50 one hour, then drastically cooling to form a martensitic structure, then reheating to about 1325° F. for not less than one hour to convert said martensitic structure into a homogeneous spheroidized cementite pearlitic structure, and again drastically cooling.

13. The method of developing in malleable cast iron, a grain having a homogeneous spheroidized cementite pearlitic structure, and having a combined carbon content of from about 0.55 percent to about 0.85 percent, a strength of about 80,000 pounds and upwards per square inch and a Brinell hardness of about 150 and upwards, which comprises subjecting malleabilized cast iron to a temperature of about 1600° F., in a carburizing 65 environment, for a time sufficient to combine with associated carbon, then drastically cooling to form a martensitic structure, then reheating to not less than 1325° F. for a time sufficient to convert said martensitic structure into a homogeneous 70 spheroidized cementite pearlitic structure, and again drastically cooling.

75

neous spheroidized cementite pearlitic structure, and again drastically cooling.

14. The method of developing in malleable cast iron, a grain having a homogeneous spheroidized cementite pearlitic structure, and having a combined carbon content of from about 0.75 percent to about 0.85 percent, a strength of about 87,000 pounds and upwards per square inch, and a Brinell hardness of about 200 and upwards,
15. which comprises subjecting malleabilized cast iron to a temperature of about 1600° F., in a carburizing environment, for not less than one hour, then drastically cooling to form a martensitic structure, then reheating to about 1325° F. for not less than one hour to convert said martensitic structure into a homogeneous spheroidized cementite pearlitic structure, and again drastically cooling.
16. A heat treated cast iron having a homogeneous spheroidized cementite pearlitic structure and substantially free from sorbitic structure, with a combined carbon content of from about 0.50 percent to about 0.85 percent, and a tensile strength of about 80,000 pounds and upwards per square inch.
17. A heat treated cast iron having a homogeneous spheroidized cementite pearlitic structure, with a combined carbon content of from about 0.50 percent to about 0.85 percent, a tensile strength of about 80,000 pounds and upwards per square inch, and a Brinell hardness of from about 150 upwards.
18. A heat treated cast iron having a homogeneous spheroidized cementite pearlitic structure and substantially free from sorbitic structure,

with a combined carbon content of from about 0.75 percent to about 0.85 percent, a tensile strength of about 87,000 pounds and upwards per square inch, a Brinell hardness of from about 200 upwards, and an elongation of about five percent, and upwards.

19. The method of heat treating malleable cast iron, which comprises heating the iron to a temperature between 1475° F. and 1600° F. to form iron carbide, quenching said iron, and reheating to a temperature of about 1325° F. for a period of time sufficient to form a spheroidized structure.

20. A heat treated cast iron product containing a major portion of the carbon in graphitic form and having a microstructure in which the matrix consists chiefly of spheroidized or globular cementite.

21. In the heat treatment of white iron to develop therein a spheroidized cementitic structure and enhanced physical properties, the steps which comprise heating such iron to a temperature above the critical for a length of time sufficient to develop in such iron a dispersion of free carbon throughout a matrix of pearlitic cementite, cooling the iron at a rate to preserve the dispersion so obtained, thereafter subjecting the iron to a temperature below but near the critical for a length of time sufficient to develop such spheroidized cementitic structure in the presence of temper carbon, and cooling the iron to room temperature.

22. An alloy formed from white cast iron by heat treatment above and below the critical in which the massive cementite originally occurring therein is in the form of temper carbon, dispersed throughout the alloy, and some of the carbon contained in the iron is in the form of spheroidized cementite dispersed through the alloy.

MAURICE G. JEWETT.  
SAMUEL C. HARRIS.